

# UNITED STATES PATENT OFFICE.

WALTER A. SCOTT, OF OAK PARK, ILLINOIS.

## ORE-CONCENTRATING PROCESS.

1,369,054.

Specification of Letters Patent. Patented Feb. 22, 1921.

No Drawing. Original application filed July 8, 1919, Serial No. 309,461. Divided and this application filed December 15, 1920. Serial No. 431,010.

*To all whom it may concern:*

Be it known that I, WALTER A. SCOTT, a citizen of the United States, residing at Oak Park, in the county of Cook and State 5 of Illinois, have invented certain new and useful Improvements in Ore-Concentrating Processes, of which the following is a specification.

My invention is an improvement in the 10 flotation process of concentrating ores when applied to ores which for efficient treatment require the presence of acid but contain considerable quantities of acid-consuming substances such as calcium carbonate or 15 other easily decomposable compound. This application is a division of my previously filed application, Serial No. 309,461, filed July 8, 1919. The usual way of introducing acid is by admixture with the pulp and the 20 acid added in this way becomes effective as a factor in the flotation process only after a quantity has been added in excess of that necessary to react with all of the easily decomposable carbonate or other substance 25 present. A quantity of the acid is wasted which is substantially the chemical equivalent of the easily decomposable substance contained in the ore. It is to avoid all, or substantially all, of this waste that I have 30 devised the method described herein.

In the treatment of ores of the type described above the effectiveness of the acid may be obtained by introducing it, preferably in gaseous form, in admixture with the 35 bubble-forming air, hydrochloric and nitric acids being among those suitable for introduction in the gaseous form. By this means the acid is brought to the bubble-water interface without coming into contact with and being uselessly consumed by 40 the carbonate or other easily decomposable substance contained in the ore, and thereby the modifying effect of the acid is obtained with a minimum consumption thereof.

45 In that form of the flotation process in which the bubble-forming air is introduced

through a permeable medium submerged in the pulp a convenient mode of procedure when hydrochloric acid is used is to cause all or a part of the air to bubble through the 50 aqueous solution of hydrochloric acid which is sold as commercial hydrochloric acid, or hydrochloric acid in the gaseous form, distilled from solution or derived from any source, may be directly mixed with the air 55 before or at the time it reaches the permeable medium. When the bubble-forming air is introduced into the pulp by agitation the upper part of the agitation cell may be enclosed except for an inlet opening through 60 which the mixture of bubble-forming air and acid may be admitted thus forming above the pulp an atmosphere of the mixture which will be beaten into the pulp in the usual way. The economies and advan- 65 tages incident to the procedure described herein are analogous to those obtained in that form of the flotation process in which the frothing and collecting agents, generally for convenience termed oils, are introduced 70 in admixture with the bubble-forming air, but in the process described herein there is an added advantage in the avoidance of wasteful acid consumption.

I claim:

1. In the flotation process of concentrating ores containing acid-consuming ingredients and in the flotation concentration of which the presence of acid improves the concentration, the operation of reducing the 80 ore to a freely-flowing pulp and introducing into said pulp a bubble-forming gas in admixture with an acid.

2. The process set forth in claim 1 further characterized by the use of acid in the 85 gaseous form.

3. The process set forth in claim 1 further characterized by the use of hydrochloric acid.

In testimony whereof, I have subscribed 90 my name.

WALTER A. SCOTT.